

# United States Patent [19]

Baldassarri et al.

[11] 3,909,268

[45] Sept. 30, 1975

- [54] **TETRAZOLIUM C-OXY-BETAINE COMPOUNDS AS ANTIFOG AGENTS FOR SILVER HALIDE PHOTOGRAPHIC EMULSIONS**
- [75] Inventors: **Agostino Baldassarri; Walter Ferro**, both of Savona, Italy
- [73] Assignee: **Minnesota Mining and Manufacturing Company**, St. Paul, Minn.
- [22] Filed: **Apr. 29, 1974**
- [21] Appl. No.: **465,185**
- [30] **Foreign Application Priority Data**  
May 7, 1973 Italy ..... 49830/73
- [52] U.S. Cl. .... 96/76 R; 96/109  
[51] Int. Cl.<sup>2</sup> ..... G03C 1/34  
[58] **Field of Search** ..... 96/109, 107, 66.5, 76 R

[56] **References Cited**  
UNITED STATES PATENTS  
3,023,103 2/1962 Dersch et al..... 96/109

*Primary Examiner*—Won H. Louie, Jr.  
*Attorney, Agent, or Firm*—Alexander, Sell, Steldt & DeLaHunt

[57] **ABSTRACT**  
Tetrazolium C-oxy-betaine compounds are effective antifog agents for silver halide photographic emulsions when reactively associated therewith. Such compounds can be incorporated in the photographic element in reactive association with the silver halide emulsion or in a processing bath prior to or during development of emulsion layers.

**17 Claims, No Drawings**

# TETRAZOLIUM C-OXY-BETAINE COMPOUNDS AS ANTIFOG AGENTS FOR SILVER HALIDE PHOTOGRAPHIC EMULSIONS

This invention relates to tetrazolium C-oxy-betaine compounds as antifog agents for silver halide photographic emulsions.

As it is known, the problem of fog, that is the silver reduced in unexposed areas upon development, is one of the most important ones to be solved in the photographic chemistry. This problem has become more critical since high temperature baths are used containing aldehydes as hardening agents.

Various compounds have long been tested and recently some good antifog agents have been described in U.S. Pat. No. 3,071,465.

We have now found that tetrazolium C-oxy-betaine compounds are very effective agents both used in a photographic element reactively associated with the silver emulsion and in a processing bath adapted for use prior to or during development of emulsion layers. They surprisingly show a very good antifogging effect with a low desensitization effect. They can also be used in combination with high temperature processing baths containing or not aldehydes as hardening agents.

The compounds useful according to the present invention are preferably those represented by the following formula:



or a mesomeric form thereof wherein R is an aryl group. In the practice of this invention, an aryl group is a phenyl group or a naphthyl group. Preferably the phenyl or naphthyl group will not contain more than a total of twelve (12) carbon atoms therein. Substituents, if any, are preferred from halogen, alkyl, alkoxy, perfluoroalkyl, haloalkyl and acyl. The substituents therefore preferably have no more than six (6) carbon atoms when attached to a phenyl ring and no more than two (2) carbon atoms when attached to a naphthyl group.

The phenyl or naphthyl ring may contain more than one of any substituent. The molecular weight of the aryl group is preferably below 300 and more preferably below 200.

- 5 Accordingly, the invention in one aspect relates to a silver halide emulsion having contacted therewith a tetrazolium C-oxy-betaine compound. In another aspect the invention relates to a silver halide photographic element having a silver halide emulsion layer and having

10 a tetrazolium C-oxy-betaine compound in reactive association therewith (e.g. in the emulsion layer or a layer adjacent the emulsion layer). The invention in a further aspect relates to a method for inhibiting fog in a silver halide photographic emulsion which comprises

15 contacting said emulsion with a tetrazolium C-oxy-betaine compound. The invention further relates to an improved method for processing an exposed silver halide element, which includes treating said element with a series of photographic treatment solutions including

20 a development solution, the improvement comprising contacting said element during said processing with a tetrazolium C-oxy-betaine compound, said compound being contained in said development solution and/or in a pre-development treatment solution. In another aspect the invention relates to a processing solution adapted for use prior to or during development of a silver photographic element, containing or not an aldehyde as hardener, containing a fog inhibiting amount of a tetrazolium C-oxy-betaine compound.

25

30 Tetrazolium C-oxy-betaine compounds as a class have been found useful as fog inhibiting agents for silver halide emulsions when reactively associated therewith. It has been found that substituents attached to nitrogen atoms do not substantially vary the capacity of

35 the compounds to inhibit fog.

Examples of tetrazolium C-oxy-betaine compounds according to the present invention are described in Table 1, which indicated their preparation methods and yields and describes their chemical-physical characteristics. Table 2 describes some prior art compounds with respect to which comparison tests have been carried out. (DMF in the above tables stands for dimethylformamide).

Table 1

| Example | R                                                                                   | m.w.   | M.P.<br>°C | Solubility |      | method | yield |
|---------|-------------------------------------------------------------------------------------|--------|------------|------------|------|--------|-------|
|         |                                                                                     |        |            | EtOH       | DMF  |        |       |
| 1       |  | 238.25 | 177        | 1.4        | 2.5  | A      | 69.8% |
| 2       |  | 307.15 | 165        | 0.5        | 2.5  | A      | 46 %  |
| 3       |  | 374.26 | 150        | 3.5        | 33.0 | A      | 35 %  |

Table I—Continued

| Example | R | m.w.   | M.P.<br>°C. | Solubility |      | method | yield |
|---------|---|--------|-------------|------------|------|--------|-------|
|         |   |        |             | EtOH       | DMF  |        |       |
| 4       |   | 335.21 | 156         | 1.8        | 6.3  | A      | 54 %  |
| 5       |   | 294.37 | 151         | 16.8       | 20.0 | C      | 48 %  |
| 6       |   | 266.31 | 165         | 6.3        | 12.5 | A      | 72 %  |
| 7       |   | 294.37 | 166         | 5.3        | 6.3  | B      | 35 %  |
| 8       |   | 391.23 | 140         | 0.33       | 10.0 | D      | 42 %  |
| 9       |   | 307.15 | 148         | 1.4        | 2.0  | D      | 38 %  |
| 10      |   | 376.05 | 140         | 0.45       | 5.0  | D      | 22 %  |
| 11      |   | 298.31 | 158         | 1.4        | 1.6  | D      | 21 %  |

Table 2

| Com-<br>pound | R | R <sub>1</sub>  | X <sup>-</sup>                | Solubility |      | method |
|---------------|---|-----------------|-------------------------------|------------|------|--------|
|               |   |                 |                               | m.w.       | EtOH |        |
| (a)           |   |                 | HSO <sub>4</sub> <sup>-</sup> | 396.43     | 3.6% | 20.2%  |
| (b)           |   | CH <sub>3</sub> | Br <sup>-</sup>               | 317.21     | 1.8% | 4.5%   |

The tetrazolium C-oxy-betaine compounds of the present invention have been prepared upon oxidation

of the corresponding c-nitro-formazanes, according to what described by A. W. Nineham, Chem. Review 55

(1955), 406 and by F. Bamberger, R. Padova, E. Ormerod, Ann. Chem. 446 (1926), 260-307. Different preparation methods have been followed corresponding to different oxidizing agents; that is to say that the herein-after illustrated methods respectively correspond to the oxidizing agents: amyl nitrite, N-bromosuccinimide, lead acetate, sodium hypochlorite. The C-nitro-formazanes have been prepared upon reaction between an aryl diazolium chloride, obtained in a conventional way, and an alkaline nitromethane solution at a temperature ranging from -15° to 0°C, in aqueous environment and in the presence of sodium acetate according to what described by E. Bamberger, R. Padova, E. Ormerod, Ann. Chem. 446 (1926) 260-307 and by D. M. Hubbard and E. W. Scott in J. A. C. S. 65 (1943) 2390.

Said methods will be hereinafter better illustrated with reference to specific examples of preparation.

#### METHOD A

##### 2,3-di-phenyl-5-oxy-tetrazolium-betaine (Example No. 1)

0.075 Moles of 1,5-diphenyl-3-nitro-formazane, 0.13 moles of amyl nitrite and 0.25 moles of acetic acid were mixed with 250 ml of acetone and refluxed on water-bath for 45'. Nitrous vapors developed from the solution and a solid separated. The whole was cooled, the solid collected by filtration and the remaining liquid still added with 0.05 moles of amyl nitrite and 0.08 moles of acetic acid. The solution was boiled for 30' to evaporate about two-thirds of the solvent. Upon dilution with ether, another solid product was prepared which was added to the aforesaid; the whole was then washed with little ether and dried under vacuum, thus obtaining a white solid under the form of shining scales. M.P. = 174°C/dec. Yield = 12.4 g equal to the 69.8% of the calculated yield. The product was then purified upon crystallization from 75% aqueous ethanol. Yield = 60%.

#### METHOD B

##### 2,3-(3,4-dimethyl-phenyl)-5-oxy-tetrazole-betaine (Example No. 7)

0.15 Moles of 1,5-(3,4-dimethyl-phenyl)-3-nitroformazane were dissolved in 600 ml of chloroform. 0.11 moles of N-bromo-succinimide were then added thereto slowly and the whole was heated up to 60°-70°C. The red solution underwent a discoloration. It was then cooled, poured into 2 l. of ether and a yellow gummy solid separated. It was crystallized first from ethanol/ether and then from 25% aqueous ethanol, thus obtaining long yellow prisms. M.P. = 166°C/dec. Yield = 35%.

#### METHOD C

##### 2,3-di-(2-ethyl-phenyl-5)-oxy-tetrazole-betaine (Example No. 5)

5 0.1 Moles of 1,5-(2-ethyl)-phenyl-3-nitro-formazane were dissolved in 300 ml of chloroform and 0.12 moles of lead tetracetate in chloroform solution added thereto slowly, thus obtaining a rich development of nitrous vapors. The whole was then refluxed for 2 h; 0.03 moles of lead tetracetate were added thereto, the solution, thus obtained, still boiled for one hour and then dried under vacuum. The residue was boiled with 800 ml of water, then cooled. The water was decanted and the remaining solid was finally crystallized first from chloroform/ether and then from 20% aqueous acetone, thus obtaining white-yellow prisms. M.P. = 151°C/dec. Yield = 48% of the calculated yield.

#### METHOD D

##### 2,3-di-(2-chloro-phenyl)-5-oxy-tetrazole-betaine (Example No. 9)

20 0.1 Moles of 1,5-(2-chloro)-phenyl-3-nitro-formazane, after pulverization, were suspended at 50°C in 350 ml of acetic acid and slowly added with sodium hypochlorite (solution: 8% active chlorine) under stirring to decolorize the formazane. 200 ml of sodium hypochlorite were necessary to decolorize completely the formazane. The whole was then cooled at 0°C, filtered upon aspiration and then poured into 10 l. of ether. The ether was cooled at 0°C, left to stand for 8 h and the crystalline solid, thus obtained, filtered. It was then washed carefully with water and dried under vacuum, thus obtaining tiny brownish needles. M.P. = 148°C/dec. Yield = 38% of the calculated yield.

#### EXAMPLE NO. 12

A silver halide photographic emulsion, containing 1.8% moles of silver iodide and 98.2% of silver bromide and having a silver-to-gelatin ratio of 1.6 was divided into several parts.

25 A part thereof (called "reference emulsion") was directly coated on a cellulose triacetate base and the other parts were added with the compounds shown in table 3 in the quantities therein specified and finally coated on a cellulose triacetate base.

30 Samples of said emulsions were then exposed under a tungsten lamp and developed for 5' at 20°C with a developer having the following composition:

|    |                            |     |   |
|----|----------------------------|-----|---|
| 50 | Methol                     | 2.2 | g |
|    | Hydroquinone               | 8.8 | g |
|    | Sodium sulfite anhydrous   | 72  | g |
|    | Potassium bromide          | 4   | g |
|    | Sodium carbonate anhydrous | 48  | g |
| 55 | Water to make              | 1   | l |

The same samples were fixed, washed and dried, then evaluated with a normal Densitometer.

Table 3

| Compound | Solvent | Quantity<br>mM/M AgX | Fresh<br>Δ Sensitivity | Fog  | incubated<br>Δ Sensitivity | Fog  |
|----------|---------|----------------------|------------------------|------|----------------------------|------|
| (a)      | DMF     | 0.05                 | -0.12                  | 0.50 | -                          | 0.53 |
| (a)      | DMF     | 0.025                | -0.08                  | 0.28 | -0.15                      | 0.25 |
| (a)      | DMF     | 0.010                | -0.06                  | 0.39 | -0.15                      | 0.40 |
| (b)      | DMF     | 0.05                 | 0.00                   | 0.39 | -0.14                      | 0.45 |
| Ex. 1    | DMF     | 0.05                 | +0.12                  | 0.45 | -0.03                      | 0.43 |
| Ex. 2    | DMF     | 2.0                  | +0.06                  | 0.18 | +0.21                      | 0.19 |
| Ex. 3    | DMF     | 0.5                  | +0.13                  | 0.21 | +0.10                      | 0.24 |
|          |         |                      |                        | 0.28 | +0.22                      | 0.33 |

Table 3 - Continued

| Compound | Solvent | Quantity<br>mM/M AgX | Fresh<br>$\Delta$ Sensitivity | Fog  | incubated<br>$\Delta$ Sensitivity | Fog  |
|----------|---------|----------------------|-------------------------------|------|-----------------------------------|------|
| Ex. 4    | DMF     | 2.0                  | -0.05                         | 0.22 | 0.00                              | 0.23 |
| Ex. 5    | DMF     | 0.5                  | +0.08                         | 0.37 | +0.16                             | 0.38 |
| Ex. 6    | DMF     | 0.5                  | +0.05                         | 0.32 | +0.08                             | 0.35 |
| Ex. 7    | DMF     | 0.5                  | +0.06                         | 0.26 | +0.09                             | 0.26 |
| Ex. 8    | DMF     | 0.5                  | -0.02                         | 0.31 | +0.02                             | 0.32 |
| Ex. 9    | DMF     | 0.5                  | 0.00                          | 0.30 | +0.03                             | 0.30 |
| Ex. 10   | DMF     | 0.1                  | -0.06                         | 0.28 | +0.03                             | 0.31 |
| Ex. 11   | DMF     | 0.5                  | -0.08                         | 0.18 | -0.10                             | 0.18 |

This table shows the sensitometric results respectively obtained with a fresh film and with a film incubated for 15 h at 72°C and 30% R.H. The sensitivity is expressed in log E. The figures shown therein are sensitivity differences ( $\Delta$  sens.) measured with respect to the reference emulsion.

## EXAMPLE NO. 13

A silver halide photographic emulsion having the same characteristics like that described in example 12 was divided into several parts. A part thereof (reference emulsion) was coated without any further addition on a cellulose triacetate base and the other parts were added with the compounds shown in Table 4 in the quantities therein specified and then coated on triacetate bases. Samples of such emulsions were exposed under a tungsten lamp and developed for 24 seconds at 35°C with a developer having the following composition:

|                                  |      |   |
|----------------------------------|------|---|
| Potassium methabisulfite         | 42   | g |
| Potassium hydrate                | 47   | g |
| Hydroquinone                     | 30   | g |
| Phenidone                        | 1.4  | g |
| Glutaraldehyde                   | 5    | g |
| Potassium bromide                | 3.9  | g |
| Water to make                    | 1    | l |
| Acetic acid to arrange the pH at | 10.1 |   |

The same samples were fixed, washed and dried, then evaluated with a normal Densitometer.

15

Table 5

| Compound | mM/l<br>Developer | g/l<br>Developer | Fog  | $\Delta$ Sensitivity |
|----------|-------------------|------------------|------|----------------------|
| Ex. 1    | 4.25              | 1.00             | 0.83 | 0.00                 |
| Ex. 2    | 2.00              | 0.612            | 1.04 | 0.00                 |
| Ex. 5    | 2.00              | 0.588            | 0.42 | 0.00                 |
| Ex. 6    | 3.76              | 1.00             | 0.63 | 0.00                 |
| Ex. 9    | 2.00              | 0.612            | 1.85 | 0.00                 |

The compounds can be introduced into the bath by using a solvent as in the case of introduction into the emulsion, or not.

30

The silver halide photographic emulsions of the present invention are silver chloride, silver bromide and silver iodide emulsions and mixtures thereof such as for example silver bromoiodide and silver chlorobromide iodide. Such emulsions may include synthetic polymeric gelatin substitutes or additives, such as dextrane, polyvinyl alcohol, polyvinyl pyrrolidone, partially hydrolyzed polyvinyl acetate, polyethylacrylate, polymethylmethacrylate, polyamides, etc. The emulsions of the invention may be chemically sensitized with naturally active gelatine, by addition of chemical sensitizers

35

Table 4

| Compound | Solvent | mM/M AgX | Fresh<br>$\Delta$ Sensitivity | Fog  | incubated<br>$\Delta$ Sensitivity | Fog  |
|----------|---------|----------|-------------------------------|------|-----------------------------------|------|
| (a)      | DMF     | 0.05     | -0.29                         | 0.67 | -0.34                             | 0.64 |
| (a)      | DMF     | 0.25     | -0.24                         | 0.57 | -0.15                             | 0.42 |
| (a)      | DMF     | 0.10     | -0.17                         | 0.59 | -0.19                             | 0.48 |
| (b)      | DMF     | 0.05     | -0.05                         | 0.57 | -0.09                             | 0.55 |
| Ex. 1    | DMF     | 0.5      | +0.03                         | 0.32 | 0.00                              | 0.30 |
| Ex. 2    | DMF     | 0.5      | -0.12                         | 0.43 | 0.00                              | 0.45 |
| Ex. 3    | DMF     | 0.5      | +0.03                         | 0.36 | 0.00                              | 0.39 |
| Ex. 4    | DMF     | 0.5      | +0.08                         | 0.43 | +0.04                             | 0.42 |
| Ex. 5    | DMF     | 2.0      | +0.06                         | 0.48 | -0.03                             | 0.45 |
| Ex. 6    | DMF     | 2.0      | +0.08                         | 0.38 | 0.00                              | 0.35 |
| Ex. 7    | DMF     | 0.5      | +0.04                         | 0.38 | 0.00                              | 0.40 |
| Ex. 8    | DMF     | 0.5      | 0.00                          | 0.35 | -0.05                             | 0.40 |
| Ex. 9    | DMF     | 0.5      | -0.08                         | 0.41 | -0.03                             | 0.41 |
| Ex. 10   | DMF     | 0.5      | -0.08                         | 0.32 | -0.1                              | 0.30 |
| Ex. 11   | DMF     | 0.1      | -0.03                         | 0.35 | -0.05                             | 0.31 |

This table shows the sensitometric results respectively obtained with a fresh film and with a film incubated for 15 h at 72°C and 30% R.H. The figures shown therein are sensitivity differences ( $\Delta$  sens.) measured with respect to their reference emulsion.

## EXAMPLE NO. 14

A photographic developer having the same composition as that described in Example 12 was divided into several parts. A part thereof was used as it was without any further addition, the other parts were each added with an antifogging compound according to our invention, as shown in Table 5. Samples of 3M X-Ray Type R materials, after exposure, were developed with such developers for 24 seconds at 35°C.

The same samples were fixed, washed and dried, then evaluated with a normal Densitometer.

Table 5 also shows the obtained results.

such as thiourea, allylthiourea, thiocyanates, thiosulfates, etc. Sensitization may be effected by the addition of noble metals, such as gold salts. Spectral sensitizers may be employed in emulsions of the invention, such as cyanine and merocyanine dyes. Moreover, the emulsions of the invention may include such additives as color couplers, filtering dyes, surfactants, hardeners, stabilizers, additional fog restrainers, plasticizers, anti-oxidizing agents, developing accelerators, etc. A photographic element comprises one support such as polyester, cellulose acetate, and the like and at least one layer including a silver halide emulsion layer of the above described type coated thereon. Such element can addi-

tionally contain other layers, that is, protective layers, interlayers, antihalo layers, filter layers, etc.

The tetrazolium C-oxy-betaine compounds of the invention may be conveniently introduced in the form of solutions into emulsions or any other coating composition during preparation thereof. Although it is generally preferred to incorporate the tetrazolium C-oxy-betaine compounds of the invention directly into emulsion layers, these compounds may also be incorporated into layers adjacent the emulsion layers so that the silver halide emulsions are again in reactive association therewith. The tetrazolium C-oxy-betaine compounds are preferably introduced into photographic elements reactively associated with the silver halide emulsions in amounts ranging from about 0.05 to 3 mM/M of silver halide and most preferably from 0.1 to 2 mM/M of silver halide.

The processing baths of the present invention, as noted previously, may be photographic pre-baths, such as those known to the art to be useful prior to treatment of a silver halide photographic element with a developing solution. Predevelopment baths are usually (but not necessarily) acidic and may contain hardeners such as aldehydes and the like. The tetrazolium C-oxy-betaine compounds of the invention may, of course, also be employed in developing baths. Such baths are normally alkaline and include one or more silver halide photographic developing agents such as hydroquinone, metol, metolhydroquinone, phenidone, hydroquinonephenidone, and various p-phenylene diamine materials, the latter being useful in color development processes. The processing baths of the invention (prebaths and developer baths) preferably include from about 1 to 10 mM/liter of solution and most preferably from 2 to 5 mM/liter of solution.

We claim:

1. A silver halide photographic emulsion having in reactive contact therewith at least a fog-inhibiting amount of a tetrazolium C-oxy-betaine compound.
2. A silver halide photographic emulsion having in reactive contact therewith at least a fog-inhibiting amount of a tetrazolium C-oxy-betaine compound corresponding to the formula



or a mesomeric form thereof wherein R is an aryl group.

3. The emulsion of claim 1 wherein said antifogging

50

compound is 2,3-di-phenyl-5-oxy-tetrazolium betaine.

4. The emulsion of claim 1 wherein said antifogging compound is 2,3-di-(4-chloro-phenyl)-5-oxy-tetrazolium betaine.

5. The emulsion of claim 1 wherein said antifogging compound is 2,3-di-(3-trifluoromethyl-phenyl)-5-oxy-tetrazolium betaine.

6. The emulsion of claim 1 wherein said antifogging compound is 2,3-di-(3-chloro-4-methyl-phenyl)-5-oxy-tetrazolium betaine.

10 7. The emulsion of claim 1 wherein said antifogging compound is 2,3-di-(2-ethyl-phenyl)-5-oxy-tetrazolium betaine.

8. The emulsion of claim 1 wherein said antifogging compound is 2,3-di-(4-methyl-phenyl)-5-oxy-tetrazolium betaine.

15 9. The emulsion of claim 1 wherein said antifogging compound is 2,3-di-(3,4-di-methyl-phenyl)-5-oxy-tetrazolium betaine.

20 10. The emulsion of claim 1 wherein said antifogging compound is 2,3-di-(2-acetyl-5-chloro-phenyl)-5-oxy-tetrazolium betaine.

11. The emulsion of claim 1 wherein said antifogging compound is 2,3-di-(2-chloro-phenyl)-5-oxy-tetrazolium betaine.

25 12. The emulsion of claim 1 wherein said antifogging compound is 2,3-di-(3,4-di-chloro-phenyl)-5-oxy-tetrazolium betaine.

30 13. The emulsion of claim 1 wherein said antifogging compound is 2,3-di-(3-methoxy-phenyl)-5-oxy-tetrazolium betaine.

14. A silver halide photographic element having a silver halide emulsion layer and a fog-inhibiting amount 35 of a tetrazolium C-oxy-betaine compound in reactive association therewith.

15. A silver halide photographic element having a silver halide emulsion layer and a fog-inhibiting amount of a tetrazolium C-oxy-betaine of formulas respectively 40 corresponding to those referred to in claims 2 in reactive association therewith.

16. The photographic element of claim 14 wherein said tetrazolium C-oxy-betaine compound is contained in said emulsion layer.

45 17. The photographic element of claims 14 wherein said tetrazolium C-oxy-betaine compound is incorporated in a layer adjacent said silver halide emulsion layer.

\* \* \* \* \*